

# UNITED STATES PATENT OFFICE.

HUGH C. SICARD, OF BUFFALO, NEW YORK.

## PROCESS FOR THE PRODUCTION OF LOW-CARBON FERROZIRCONIUM.

1,374,037.

Specification of Letters Patent.

Patented Apr. 5, 1921.

No Drawing.

Application filed July 23, 1920. Serial No. 398,512.

To all whom it may concern:

Be it known that I, HUGH C. SICARD, a citizen of the United States of America, and a resident of the city of Buffalo, county of Erie, and State of New York, have invented a certain new and useful Process for the Production of Low-Carbon Ferrozirconium, of which the following is a full, clear, and exact description.

10 In general this invention relates to a method or process of manufacturing and producing a low carbon ferro-zirconium and more particularly to a ferro-zirconium alloy preferably having a carbon content of less than two per cent.

On June 1st, 1920, Letters Patent No. 1,341,939 were granted me on a process for the production of low carbon ferro-chrome. The process or method herein described is in 20 some respects like that described in the said Letters Patent. That process, however, has been modified in the manner hereinafter set forth in order to apply it to the manufacture of low carbon ferro-zirconium.

25 In seeking to produce low carbon ferro-zirconium heretofore, those skilled in the art have sought to decarbonize the ferro-zirconium by using a zirconium ore in combination with burnt lime; the lime in such case forms a protective blanket of slag over the molten metal. The zirconium ore then reacts with the ferro-zirconium which contains carbon and in time the zirconium ore is decarbonized. A great objection to this proc-

35 ess resides in the fact that the iron oxide which is present in the zirconium ore is more readily reduced than the oxide of zirconium with the result that when the final substantially decarbonized ferro-zirconium is obtained it is found to have a lower content of 40 zirconium than the original high carbon material.

In the invention herein described, I have overcome the difficulties above set forth.

45 In carrying out my invention, I use titanic oxide ( $TiO_2$ ) for the purpose of decarbonization. This oxide reacts with the carbon in the high carbon ferro-zirconium and forms titanium.

50 As a source of the titanic oxide, it is quite important that there be used some ore which contains a very small amount of iron oxide. For this purpose I preferably use rutile.

The reaction is carried out, preferably 55 in an electric furnace of the well known arc type. In this furnace is charged a mixture

of the alloy of ferro-zirconium which has a certain carbon content and a quantity of rutile which will be sufficient to decarbonize the alloy used. In place of the ferro-zirconium I may use an alloy of zirconium and titanium which is high in carbon and then decarbonize it by the same process as hereinbefore set forth. Into this a charge of burnt lime is placed and melted down. The 65 burnt lime forms a protective slag and when the reaction is complete the resulting alloy is tapped from the furnace.

Obviously, instead of following the process exactly as hereinbefore set forth, the 70 high carbon alloy could be first melted with a blanket of lime and then the titanic oxide could be added as the decarbonizing element.

Having thus described my invention, what I claim is:

75 1. The method of making a low carbon alloy of iron and zirconium which consists in the decarbonization of a high carbon ferro-zirconium alloy by means of titanic oxide.

80 2. The method of making a low carbon alloy of iron and zirconium which consists in the decarbonization of a high carbon ferro-zirconium alloy by means of an ore high in titanic oxide and low in iron oxide. 85

3. The method of making a low carbon alloy of iron and zirconium which consists in the decarbonization of high carbon ferro-zirconium alloy by means of rutile ore.

4. The method of making a low carbon 90 alloy of iron and zirconium which consists in charging into an electric furnace a mixture of ferro-zirconium, high in carbon, and a sufficient quantity of titanic oxide to decarbonize the alloy.

95 5. A method of making low carbon alloys of iron and zirconium which consists in charging into an electric furnace a mixture of ferro-zirconium which is high in carbon and a sufficient quantity of rutile to decarbonize the alloy. 100

105 6. The method of making a low carbon alloy of iron and zirconium which consists in charging into an electric furnace a mixture of ferro-zirconium which is high in carbon, a sufficient quantity of titanic oxide to decarbonize the alloy and a sufficient quantity of burnt lime to form a protective slag.

In testimony whereof, I have hereunto signed my name.

HUGH C. SICARD.